

## UNITED STATES PATENT OFFICE

2,344,495

## NONSTAINING COATED FABRIC

Merle H. Chamberlin, Newburgh, N. Y., assignor  
to E. I. du Pont de Nemours & Company,  
Wilmington, Del., a corporation of Delaware

No Drawing. Application October 25, 1941,  
Serial No. 416,601

1 Claim. (CL 117—86)

This invention relates to cellulose derivative coated fabrics which may be readily cleaned of stains resulting from colored cosmetics, foodstuffs, etc., and more particularly to cellulose nitrate coated fabrics having a surface coating of a cellulose derivative resistant to permanent staining.

At the present time cellulose nitrate coated fabrics have achieved widespread use in the manufacture of ladies' handbags or pocketbooks as a result of the long wearing qualities and the unique combinations of grains and colors to which the material is adapted. In the ladies' pocketbook field, the coated fabric is used both as an outside covering as well as an inside lining material. As far as initial appearance and wearing qualities are concerned, these materials have been accepted by the trade as being satisfactory. The cellulose nitrate coated fabrics are produced in an unlimited variety of colors, grains and finishes which are generally considered to be "washable" since the coating is not water soluble. However, improvement is desired in the case of white and pastel shades which are employed in making ladies' pocketbooks for use during the spring and summer seasons, since the lighter shades become readily soiled by colored cosmetics, such as lipstick, rouge, face powder, etc. Such stains cannot be removed from the surface of the nitro-cellulose coatings by conventional cleaning methods available in the home which employ soap and water, carbon tetrachloride, and commercial dry cleaning fluids. Once a white or pastel shade pocketbook, made from nitrocellulose coated fabrics, becomes soiled by colored cosmetics it is usually considered unusable since such stains cannot be readily removed and the pocketbook is discarded.

White and light colored cellulose nitrate coated fabrics are also extensively used as a table cover instead of untreated linen. The nitrocellulose coated fabric table covers are considered washable and are accepted by the trade as being satisfactory as regards initial appearance and wearing qualities. However, there is further improvement desired in this type of product with respect to resistance to permanent staining by foodstuffs, such as, e. g., cocoa, catsup, coffee, turmeric, prepared mustards, fruit juices, fats, oils, etc.

As a result of a great deal of research on the permanent stain resistance of various film forming materials, several were found which permitted removal of stains resulting from the materials mentioned above. However, many of the film forming materials which permitted the ready re-

moval of such stains, include polyvinyl alcohol, zein, "Vinylite" resins, and cellulose acetate; these materials, however, will not satisfactorily anchor to pyroxylin surfaces without special intermediate bonding coats with resulting increases in cost of manufacture. Film-forming materials which will readily anchor to cellulose nitrate, include cellulose nitrate, nylon, ethyl cellulose, and gelatin; these materials, however, are not resistant to permanent staining by colored cosmetics and foodstuffs. The desideratum is a film-forming substance which will readily anchor to a pyroxylin surface without intermediate bonding substance and which may be readily cleaned from stains resulting from colored cosmetics, foodstuffs, etc.

This invention therefore has as a primary object the minimization or elimination of the aforesaid disadvantages inherent in products or coatings consisting essentially of nitrocellulose compositions, while at the same time preserving and utilizing the aforesaid advantageous properties thereof. More particularly the object is to provide a surface coat which will anchor satisfactorily to nitrocellulose and at the same time be resistant to lipstick and the like.

This object, as well as other important but subsidiary objects which will become apparent as the description of the invention proceeds, is accomplished according to the invention by applying directly to a nitrocellulose containing base, a surface coating consisting essentially of a cellulose aceto propionate or cellulose aceto butyrate as the film-forming ingredient. The term directly implies no intermediate anchoring coat.

The following is one embodiment given by way of illustration and not limitation; it being understood that the invention is not limited thereto.

## EXAMPLE I

40 To a woven cotton fabric running 1.32 yards per pound per 53" width and having a sateen weave was applied a plurality of coats of a cellulose nitrate coating of the following approximate composition, by means of a doctor knife:

## Base coating composition

|                   | Per cent by weight |
|-------------------|--------------------|
| Cellulose nitrate | 14.10              |
| White pigment     | 14.57              |
| Castor oil        | 24.76              |
| Ethyl alcohol     | 23.28              |
| Ethyl acetate     | 23.29              |

45 The method of preparing the above composition is well known in the art. The volatile sol-

vents were expelled between each successive coat of the composition by passing the material through a heated chamber. Sufficient coats of the above composition were applied to deposit approximately 15 ounces of the non-volatile components on each yard of fabric per 50" width. The material was given an intermediate embossing treatment at the half-way stage of coating operation by passing it between heated pressure rolls.

The thus-treated material was given one or more final coats of the following composition:

*Surface coating composition*

|                                 | Per cent by weight |
|---------------------------------|--------------------|
| Cellulose aceto propionate      | 18.75              |
| Ethyl phthallyl ethyl glycolate | 6.25               |
| Ethyl alcohol                   | 37.50              |
| Ethyl acetate                   | 37.50              |

The volatile solvents were expelled by passing the coated fabric through a heated chamber. The material had a bright, glossy finish as it emerged from the drying chamber and the surface coating was firmly anchored to the nitrocellulose coating. Sufficient surface coating composition was applied to deposit approximately 1 to 2 ounces of non-volatile components per yard per 50" width. The thus-treated material was next ornamented by embossing treatments. Either the roller or plate type embossing may be employed. Depending upon the appearance desired in the finished product, the embossing operation may or may not be followed by the application of the additional coat of the non-staining surface coating before the material is made up into ladies' handbags.

*EXAMPLE II*

A coated fabric was also prepared in the same manner as described in Example I except the final surface coating composition was as follows:

|                   | Per cent by weight |
|-------------------|--------------------|
| Cellulose nitrate | 12.35              |
| Ethyl alcohol     | 43.82              |
| Ethyl acetate     | 43.83              |

The coated fabrics prepared in accordance with Examples I and II were identical in appearance, color, luster and had similar wearing qualities. Both coated fabrics were stained with red lipstick (indelible), purple duplicating pencil, black carbon paper, red wax pencil (crayon), prepared mustard, coffee, cocoa, catsup, mercurochrome and merthiolate, and allowed to stand over night; the stains on the cellulose nitrate surfaced material could not be removed when rubbed with a cloth saturated with known solvents for the coloring materials which are non-solvents for the nitrocellulose; such as carbon tetrachloride, benzene, 50-50 mixture of benzene and carbon tetrachloride, ethyl alcohol, water, etc. Likewise the stains on the nitrocellulose surface could not be removed when scrubbed with soap and water, or rubbed vigorously with a dry cloth.

On the other hand, the cellulose aceto propionate surfaced material was readily cleaned free of all colored stains produced with the materials mentioned above by rubbing the stains with a cloth saturated with any one of the following solvents which are non-solvents for the cellulose aceto propionate; such as carbon tetrachloride, ethyl alcohol, benzene, toluol, water, and a mixture of equal parts of carbon tetrachloride and benzene. The colored stains were

also removed with the aid of soap and water alone. Practically all of the stains are removed with the aid of a dry cloth but a slight trace of color remained which was readily removed by the solvents mentioned above.

When the colored markings were allowed to remain on the coated fabrics for a period of two weeks before attempting to remove them, as in the case where the stains were allowed to remain on the coated fabrics over night, none of the stains could be removed from the nitrocellulose surfaced material, whereas the two week old stains were all readily removed from the cellulose aceto propionate surfaced material with the aid of any of the solvents for the coloring matter which are non-solvents for the cellulose aceto propionate, which are mentioned above. The two week old stains on the cellulose aceto propionate surfaced material were also readily removed with the aid of soap and water.

Instead of the cellulose aceto propionate composition described in the preferred embodiment equally good results have been obtained with the following composition when applied as a surface coat over a pyroxylin containing base material.

*EXAMPLE III*

|                                                      | Percent by weight |
|------------------------------------------------------|-------------------|
| Cellulose aceto butyrate                             | 18.75             |
| Mixture of ortho and para toluene ethyl sulfonamides | 6.25              |
| Ethyl alcohol                                        | 37.50             |
| Ethyl acetate                                        | 37.50             |

*EXAMPLE IV*

Another modification of the invention employs the use of pigments in the final surface coat to produce satin, mat or dull finish effects. This modified form is accomplished by applying to a nitrocellulose coated fabric base prepared in the same manner as described in Example I the following composition as a final surface layer either before or after embossing operation:

|                                                     | Percent by weight |
|-----------------------------------------------------|-------------------|
| Cellulose aceto propionate                          | 17.90             |
| Zinc oxide                                          | 13.84             |
| Mixture of ortho and para toluene ethyl sulfonamide | 6.92              |
| Ethyl alcohol                                       | 30.67             |
| Ethyl acetate                                       | 30.67             |

Coated fabrics having surface coats as described in Examples III and IV possessed the same resistance to permanent staining as did the material described in Example I.

*EXAMPLE V*

Still another modification of the invention is the production of a highly glazed, readily cleanable, coated fabric resistant to piping, having a nitrocellulose base coating and a surface coating deposited from the following coating composition:

|                                | Percent by weight |
|--------------------------------|-------------------|
| Cellulose aceto propionate     | 13.12             |
| Triethylene glycol dicaprylate | 24.68             |
| Ethyl alcohol                  | 31.10             |
| Ethyl acetate                  | 31.10             |

The highly glazed coated fabric which is resistant to permanent staining has the added advantage of being resistant to piping, herein-after more fully explained.

While the invention has been described with respect to a specific construction of coated fabric designed for use as a lady's pocketbook, it will be readily apparent to those skilled in the

art that the invention can be utilized with any pyroxylin coated fabric construction or pyroxylin surfaced material which may be flexible or rigid. There is no limitation to be placed upon the composition of the pyroxylin material which may be surfaced in accordance with the teachings of this invention.

The plasticizer for the cellulose aceto propionate or cellulose aceto butyrate is preferably one which is not a solvent for such waxes as ceresin and stearic acid which are commonly used in lipsticks, wax pencils, etc. Plasticizers for the cellulose aceto propionate or cellulose aceto butyrate other than those mentioned in the examples which have been found to be satisfactory for the purpose of this invention are triethylene glycol dihexoate, dibutyl tartrate and triethylene glycol dicaprylate.

It has been found that the stain retention of the surface layer is in proportion to the amount of plasticizer content present in the surface layer. It has been discovered that if the plasticizer content of the surface coat is increased beyond 65% of the total amount of non-volatile components of the surface layer, that the stains produced by colored cosmetics, food-stuffs, and the like, are not as easily removed as materials having a lower plasticizer content.

In the case of coated fabrics which are to be subjected to pleating, such as in the construction of certain types of ladies' handbags, it is necessary to employ to very supple film as the outer layer of the coating to prevent "piping" on an inside fold of the coated fabric. The term "piping" refers to a crinkling effect consisting of a series of fine parallel lines. When bent or folded the "piping" is caused by a difference in elasticity of the nitrocellulose base coating and the non-staining cellulose aceto propionate or cellulose aceto butyrate surface coat. Therefore, it is desirable to employ as much plasticizer in the non-staining surface coat as is consistent with stain resistance on materials which are to be subjected to folding or bending.

There is no limitation on the pigments to be used in practicing this invention which be any single pigment, or mixture of pigments, to produce the desired shade.

While the invention has been described with respect to the manufacture of material to be used for ladies' handbags both as an outer cover and inside lining, as well as lacquered table-

cloths, the products of the invention will also find great utility in other fields. The ready removal of colored cosmetic stains from the coated fabric makes it particularly useful as an optical case covering, since such cases are frequently carried in ladies' handbags and are susceptible to becoming stained with colored cosmetics. Another important field in which the products of the invention are useful is the lacquered wall covers for kitchen installation, since stains resulting from foodstuffs are readily removed with the aid of soap and water. Still another important use for the product of this invention is for mattress covers and hospital upholstery due to the ready removal of stains which are normally encountered in the use of such material.

The outstanding advantage of the material produced in accordance with the teachings herein is the ready removal from the coated fabrics of stains produced by colored cosmetics such as, e. g., lipstick, rouge, face powder, etc., as well as the ready removal of food stains, such as, e. g., prepared mustard, cocoa, coffee, catsup, turmeric, fats, oils, fruit juices, etc. Other important advantages will be readily apparent to those skilled in the art of coated fabrics.

It is apparent that many widely different embodiments of this invention may be made without departing from the spirit and scope thereof, and therefore, it is not intended to be limited except as indicated in the appended claim.

I claim:

A light colored coated fabric adapted for making handbags and the like and which is highly resistant to permanent staining by colored cosmetics and foodstuffs which comprises a base fabric having a coating of a composition weighing approximately 15 ounces of non-volatile material per yard of 50 inch width fabric, the film-forming ingredient of the said composition consisting essentially of cellulose nitrate and in contact with the said composition a surface coating containing about 3 parts of a mixed ester of cellulose selected from the group consisting of cellulose acetopropionate and cellulose acetobutyrate and about 1 part of a solvent plasticizer therefor, said surface coating being present in the amount of about 1 to 2 ounces of non-volatile components per yard of 50 inch width material.

MERLE H. CHAMBERLIN.